

April 2, 1946.

R. P. HEUER

**2,397,737**

## PROCESS OF DESULPHURIZING

Filed July 14, 1942

4 Sheets-Sheet 1



## Inventor.

*Russell Pearce Heuer.*

by John Steele Jackson and Sons  
Attorneys.

Witness:  
Walter Chum.

April 2, 1946.

R. P. HEUER

2,397,737

PROCESS OF DESULPHURIZING

Filed July 14, 1942

4 Sheets-Sheet 2



Inventor  
Russell Pearce Heuer

by John Stuckeljahn and Son

Attorneys

Witness:  
Walter Chinn

April 2, 1946.

R. P. HEUER

2,397,737

PROCESS OF DESULPHURIZING

Filed July 14, 1942

4 Sheets-Sheet 3



Witness:  
Walter Chinn.

Inventor  
Russell Pearce Heuer  
by *John Stetzel, Jr. and Son*  
Attorneys.

April 2, 1946.

R. P. HEUER

**2,397,737**

## PROCESS OF DESULPHURIZING

Filed July 14, 1942

4 Sheets-Sheet 4

Fig. 16.



Fig. 15.



Fig. 20.



## Inventor.

Russell Pearce Hener.

by J. Steel Jackson and Son

## Attorneys.

Witness:  
Walter Cherry

## UNITED STATES PATENT OFFICE

2,397,737

## PROCESS OF DESULPHURIZING

Russell Pearce Heuer, Villa Nova, Pa., assignor  
to Essex Research Corporation, Wilmington,  
Del., a corporation of Delaware

Application July 14, 1942, Serial No. 450,892

5 Claims. (Cl. 75—55)

My invention relates to a process for the treatment of pig iron and the production of steel and principally to the desulphurization of pig iron. This application is a continuation in part of my copending applications, Serial No. 304,484, filed November 15, 1939, and Serial No. 374,989, filed January 18, 1941, for Desulphurizing apparatus and process.

A purpose of the invention is to operate a coke blast furnace to produce pig iron higher in sulphur than that ultimately desired, and preferably at a lower cost than normal, by operating the blast furnace at a lower temperature and/or with less basic slag and/or with low grade raw materials causing higher sulphur in the charge, and to provide improved apparatus in which to treat the molten pig iron thus produced with a basic slag external to the blast furnace hearth, to remove the excess sulphur from the molten pig iron. The pig iron thus produced may be used in the form of cast iron or as raw material for making steel.

A further purpose is to remove molten pig iron at periodic intervals from the blast furnace, to transfer it in molten state by a runner or other suitable mechanism to a fore-hearth or ladle adjoining the blast furnace in such a way as to prevent undesirable amounts of silica and other contaminating substances present in the runner from entering the desulphurizing forehearth, subjecting the molten pig iron in the forehearth to desulphurizing action and transferring the desulphurized iron to a transfer ladle for subsequent use in the manufacture of steel, or other purposes.

A further purpose is to desulphurize pig iron in a suitable forehearth or ladle adjacent to the blast furnace, to separate the molten pig iron from the desulphurizing slag and to deliver the desulphurized pig iron free from desulphurizing slags to a transfer ladle for conveying the molten iron to steel making furnaces.

A further purpose is to desulphurize molten pig iron by means of a slag in a forehearth or ladle adjacent to a blast furnace or other furnace capable of providing molten iron, the forehearth or ladle having its axis of symmetry in a substantially vertical position and provided with means for producing a rotary motion of the contents of the forehearth or ladle about the axis of symmetry.

A further purpose is to place molten iron in the refractory lining of a desulphurizing ladle whose axis of symmetry is vertical, with a basic desulphurizing slag floating on the molten iron, and impart rotary motion to the metal, desirably in a horizontal plane, while desirably also producing relative movement between the slag and the iron.

A further purpose is to rotate molten iron or

basic desulphurizing slag in contact with the iron by an impeller or preferably a plurality of impellers turning on a vertical axis and preferably in a ladle whose axis of symmetry is vertical. The impellers will preferably turn in the same direction.

A further purpose is to employ a plurality of impellers operating in contact with molten iron, and a basic desulphurizing slag on the molten iron, at different levels, one effective below the slag-metal interface and another effective at or above the interface.

A further purpose is to rotate molten iron in the presence of a supernatant slag in a ladle having its axis of symmetry substantially vertical and to produce a relative movement between the slag and metal, to facilitate the transfer of impurities from the metal to the slag, by means of a dam or obstruction which impedes the flow of the slag whilst permitting greater flow of the metal.

A further purpose is to obtain relative movement between molten iron and desulphurizing slag floating on the molten iron by means of a dam in contact with the slag and adjustable with respect to the level of the slag-metal interface. The dam may be rigidly positioned or floating and if floating, it will desirably be flexibly restrained.

A further purpose is to rotate molten iron in the presence of a supernatant slag in a ladle having its axis of symmetry substantially vertical and to produce from the rotary movement of the iron, a vertical motion in the iron to bring the impurities in the iron into contact with the slag.

A further purpose is to obtain a vertical component of rotary motion imparted to molten iron having desulphurizing slag floating on the molten iron, by an upwardly inclined vane preferably of helical character in the refractory lining containing the iron.

A further purpose is to agitate molten pig iron in the presence of a slag by means of a rotating impeller capable of raising the molten pig iron above the normal level of the slag-pig iron interface.

A further purpose is to lift molten iron into contact with a basic desulphurizing slag by a pumping impeller having an upwardly and outwardly inclined passage whose inlet is below the slag-metal interface and whose outlet is above the interface.

A further purpose is to employ a refractory impeller having one or preferably a plurality of flat preferably vertical surfaces and rotating about a substantially vertical axis.

A further purpose is to employ a refractory impeller for stirring molten metal having a pref-

erably helical groove in an outer surface of generally cylindrical character.

A further purpose is to render a stirring or pumping impeller of refractory material adjustable as to level by connecting the impeller to the impeller shaft through an impeller extension which can be replaced by an extension of different length.

A further purpose is to promote reaction between molten metal and a desulphurizing slag floating on the molten metal by imparting horizontal rotatory motion to the charge in a desulphurizing vessel whose axis of symmetry is vertical and whose horizontal cross section is oval.

A further purpose is to agitate molten pig iron in the presence of a supernatant slag in a ladle by means of electromagnetic action.

A further purpose is to whirl a pig iron bath by horizontal rotary electromagnetic stirring and to maintain a substantial body of molten desulphurizing slag on the bath, the slag permissibly rotating with the iron but preferably being dammed against rotation or more desirably being oppositely rotated.

A further purpose is to impart an electromagnetic stirring motion, preferably in a horizontal rotary direction, to molten pig iron on which a substantial body of desulphurizing slag is floating, and to induce an upward stirring component in the iron preferably by an inclined vane.

A further purpose is to produce agitation in molten pig iron in contact with a supernatant desulphurizing slag by electromagnetic flux from a multiphase winding surrounding the iron and provided with a ring-like magnetic core, the winding and/or core being inclined to the horizontal so as to produce helical stirring components.

A further purpose is to avoid contamination of silica and siliceous materials with molten iron drawn from a blast furnace or similar source of molten iron to an adjacent desulphurizing vessel, by passing the molten iron through a skimming ladle or other means for separating siliceous impurities.

A further purpose is to employ a desulphurizing vessel having a slag tap opening and a metal tap opening on opposite sides and to pour slag by tilting the vessel on a tilting axis adjacent the slag top opening and to pour metal by tilting the vessel on a tilting axis adjacent the metal tap opening.

Further purposes appear in the specification and in the claims.

The invention relates both to the apparatus for treating the molten metal and to the processes therefor.

The present application incorporates by reference my United States patents and patent application, Patent No. 2,110,066, granted March 1, 1938, for Iron and steel desulphurization; Patent No. 2,110,067, granted March 1, 1938, for Iron desulphurization; Patent No. 2,177,716, granted October 31, 1939, for Desulphurizing apparatus; Patent No. 2,193,593, granted March 12, 1940, for iron desulphurization; and Serial No. 304,484, filed November 15, 1939, for Desulphurizing apparatus and process. It is the purpose and intent that subjects matter may be transferred from this application to the present application as required. Reference should be had to these patents and this application for further disclosure of the process.

In the drawings no attempt has been made to illustrate all of the possible embodiments of the

invention. The forms shown have been chosen from the standpoints of satisfactory operation and convenient illustration of the principles involved. All of the figures are diagrammatic.

Figure 1 is a diagrammatic central vertical section of a desulphurizing vessel in accordance with the present invention, with cooperating structure.

Figure 1a is a fragment of Figure 1 showing covers applied over the openings.

Figure 2 is a central vertical section of one form of stirring impeller in accordance with the invention.

Figure 2a shows a different length of impeller extension from that shown in Figure 2.

Figure 3 is a side elevation of a variant form of stirring impeller in accordance with the invention.

Figure 4 is a side elevation of a further variant form of stirring impeller.

Figure 5 is a section of Figure 4 on the line 5-5.

Figure 6 is a diagrammatic central vertical section of a modified form of desulphurizing vessel.

Figure 7 is a section of Figure 6 on the line 7-7.

Figure 8 is a central vertical section of a further modification in the desulphurizing vessel.

Figure 9 is a section of Figure 8 along the line 9-9.

Figure 10 is a fragment showing a modified form of dam applied to the structure of Figure 8.

Figure 11 is a fragmentary top plan view of Figure 10.

Figure 12 is a fragmentary central vertical section showing a further modification in the dam of Figure 8.

Figure 13 is a central vertical section of a further modification in the desulphurizing vessel.

Figure 14 is a section of Figure 13 on the line 14-14.

Figure 15 is a side elevation of a modified form of desulphurizing vessel with an electrical diagram of a polyphase inductor coil applied thereto, the magnetic core being sectioned away for convenience in illustrating the coil.

Figure 16 is a section of Figure 15 on the line 16-16.

Figure 17 is a diagrammatic top plan view of a variant form of electromagnetic stirring ladle.

Figure 18 is a fragmentary side elevation of Figure 17.

Figure 19 is a diagrammatic horizontal section of a modified desulphurizing vessel.

Figure 20 is a curve showing the rate of sulphur removal from pig iron under special controlled conditions.

In the drawings like numerals refer to like parts, and in the specification like symbols refer to like subjects matter.

Throughout the specification, wherever reference is made to pig iron, it is intended to designate the product of the blast furnace which characteristically has a high carbon content, usually of 3% to 4%, or more, and always in excess of 2%, with varying contents of metalloids. The product of the blast furnace is referred to as pig iron whether it is intended to be used in the form of cast iron or whether it is to be used in making steel.

In the production of pig iron from low-sulphur burdens (such as wood charcoal and low sulphur ores) it is unnecessary to operate the blast furnace in such a manner as to obtain strong desulphurizing conditions in the hearth and bosh

of the blast furnace. As a result the operation of the charcoal blast furnace is quite economical except for the excessive costs of wood charcoal and of low sulphur ores. In most instances, however, because of the high cost of wood charcoal, it is necessary to substitute coke for wood charcoal as a blast furnace fuel. When this is done, a strong desulphurizing action must be obtained in the hearth and bosh of the blast furnace in order to obtain a product having low enough sulphur to be commercially usable. For a strong desulphurizing action, it is necessary to have a higher temperature and a slag containing more lime than for a weaker desulphurization. More fuel must be used in order to provide the higher temperature.

A typical slag from a charcoal blast furnace approximates:

|                                | Percent | 20 |
|--------------------------------|---------|----|
| SiO <sub>2</sub>               | 47.0    |    |
| Al <sub>2</sub> O <sub>3</sub> | 18.0    |    |
| CaO                            | 27.0    |    |
| MgO                            | 3.0     |    |
| S                              | 0.10    |    |

In the above slag the silica exceeds the lime plus magnesia. The sulphur in the pig iron approximates 0.02%.

A typical slag from a coke blast furnace has the following approximate composition:

|                                | Percent | 30 |
|--------------------------------|---------|----|
| SiO <sub>2</sub>               | 34.0    |    |
| Al <sub>2</sub> O <sub>3</sub> | 12.0    |    |
| CaO                            | 40.0    |    |
| MgO                            | 10.0    |    |
| S                              | 1.7     |    |

In the above slag the silica is less than the lime plus magnesia. The sulphur in the pig iron approximates 0.03%.

The temperatures of the slag and pig iron tapped from a charcoal blast furnace are about 1450° C. and 1410° C. respectively. In the coke blast furnace, the respective temperatures of the slag and pig iron as tapped are approximately 1525° C. and 1475° C. Thus it is unnecessary for the charcoal blast furnace to expend as much heat to produce slag and pig iron as does the coke blast furnace.

From the above data it will be obvious that the cost of removing sulphur from the pig iron simultaneously with smelting of the ore in a blast furnace is considerable. It is one purpose of the present invention to cheapen the cost of manufacturing pig iron, whether for use as cast iron or for making steel, by omitting the strong desulphurizing action now considered necessary in the coke blast furnace because of the sulphur-bearing burdens. The smelting is conducted in the coke blast furnace under conditions of temperature and basicity of slag suitable to produce pig iron at lower cost but with a higher sulphur content in the iron than that ultimately desired. The sulphur content in the iron produced may be for example 0.25% sulphur. After production of this high sulphur pig iron by the invention, it is treated as a wholly independent operation to remove the excess of sulphur. The cost of the desulphurization is small and it is possible to produce pig iron of desirable quality at a considerable saving. Of course, it is not necessary that the high sulphur pig iron contain as much as 0.25% sulphur before treatment. The process is equally adapted to the desulphurization of pig

iron containing 0.10% sulphur or 0.05% sulphur or less depending upon individual conditions.

The pig iron, containing a higher sulphur content than that ultimately desired, is transferred from the coke blast furnace to a suitable desulphurizing vessel as described later. The pig iron is there subjected to a strongly basic slag under reducing conditions.

The desulphurizing slag contains basic oxides of the alkaline earth or alkali metals such as calcium oxide, barium oxide, strontium oxide, sodium oxide, etc. These are referred to generically as R<sub>x</sub>O oxides, where R is an alkaline earth or alkali metal and x is the numeral 2 or 1, depending upon the valence of the metal. The oxides of the slag tend to react with sulphur of the pig iron thus:



From reactions 1 and 2 it will be evident that there will be a low activity of sulphur and sulphur can be removed from the pig iron to enter the slag most efficiently if there is a low oxygen activity. In other words, the sulphur activity may be lowered directly by lowering the oxygen activity. The desulphurizing slag is, therefore, caused to act upon the pig iron in the presence of a deoxidizing agent, as for example an excess of carbon preferably under diminished pressure, or in the presence of carbon compounds such as calcium carbide or metallic reducing agents such as manganese, silicon, aluminum, calcium, magnesium or the like. There will, of course, very desirably be substantially complete exclusion of oxygen and oxidizing substances from the desulphurizing vessel, by suitable closures, seals, gaskets and the like.

The pig iron desulphurized by the present invention will in most cases be pig iron produced in the coke blast furnace when operated under conditions of moderate temperature and moderate basicity of the slag suitable to produce pig iron of lower cost but with a higher sulphur content than that ultimately desired. Ore of low iron content and coke or ore of high sulphur content may be used. The sulphur content of the pig iron produced in the coke blast furnace under such economical conditions may be 0.25%, 0.3% or even higher. Of course, the invention may also be applied to pig iron of normal sulphur content, containing, say 0.04% S.

The pig iron to be desulphurized is brought into contact with a desulphurizing slag under the proper conditions. For example, the desulphurizing slag can first be charged into a ladle or other vessel and the molten iron can then be added.

#### Slags

The preferable slag will have CaO as its active desulphurizing oxide. As previously explained, other alkaline earths or alkaline oxides can be used. The inventor has found, however, that CaO is very desirable and economical as a desulphurizing agent and it will be used in many of the illustrations, although quite evidently other oxides described could be used in similar manner after making due allowance for known differences in physical and chemical properties of the other oxides.

CaO in the pure state has a high melting point (2570° C.). It is conventional to reduce the melting point of CaO to form readily fusible slags by adding SiO<sub>2</sub> and perhaps Al<sub>2</sub>O<sub>3</sub> and other oxides.

Thus, for example, it is possible to form a slag which is free-flowing at 1400° C. having the approximate composition:

|                                | Percent |
|--------------------------------|---------|
| CaO                            | 44      |
| MgO                            | 4       |
| Al <sub>2</sub> O <sub>3</sub> | 15      |
| SiO <sub>2</sub>               | 37      |

In such a slag the activity of the lime is reduced by the presence of 37% silica and 15% alumina. Slags of this approximate composition are used as desulphurizing agents in the blast furnace and are capable of building up a 60:1 ratio of the percentage of sulphur in the slag to the percentage of sulphur in the pig iron. It has been found that such a slag can be used in the present invention, especially if the slag and pig iron to be desulphurized are subjected to a diminished pressure, desirably 150 millimeters of mercury or less, and in the substantial absence of oxygen and oxidizing substances, thereby causing the sulphur ratio to rise to 100:1 or 200:1 or more, depending upon specific conditions.

If ordinary blast furnace slag is used, it may desirably be mixed with say 5% to 10% or even 20% or more by weight of fluorspar and, if desired, up to 20% or more by weight of burned lime or substances high in CaO such as burned dolomite or dolomitic lime. About 2% of lime is the minimum lime addition which is substantial in effect. The lime content of the slag should not exceed 55%. A typical mixture might consist of 70% blast furnace slag, 10% fluorspar, 20% lime. Such a slag when held in contact with pig iron of high sulphur content (0.16% S) at 1400° C. in a non-oxidizing atmosphere, at normal pressure, reduced the sulphur content of the iron to 0.015% S and the slag increased its sulphur content to 2.66%. A similar slag under an absolute pressure of 35 millimeters of mercury reduced the sulphur content of the iron to 0.001% and the slag contained 2.83% sulphur.

Blast furnace slag mixed with lime and/or fluorspar as just explained, may be employed in any of the forms of the invention disclosed herein in whether the deoxidizing agent be carbon at atmospheric pressure or at reduced pressure, or other deoxidizing agent as explained above.

Where carbon is the deoxidizing agent, it may in some cases be supplied by the carbon dissolved in the pig iron, which normally contains more than 2% of carbon, and in other cases this dissolved carbon may be supplemented by a carbon lining in the reaction vessel and/or by loose carbon added to the reaction vessel.

The SiO<sub>2</sub> content of the desulphurizing slag can also be further decreased, and slags have been synthesized containing as little as 15% SiO<sub>2</sub> or less, as for example using a mixture of 40 parts blast furnace slag, 30 parts fluorspar, 30 parts lime, which slag would contain about 12% SiO<sub>2</sub>. It has been found that such slags are very advantageous especially where the slag and pig iron under treatment cannot be subjected to low pressures.

A desulphurizing slag having the composition:

|                  | Percent |
|------------------|---------|
| CaO              | 45      |
| CaF <sub>2</sub> | 40      |
| SiO <sub>2</sub> | 15      |

has also been found to be very satisfactory. Such a slag can be readily synthesized by mixing lime and fluorspar of commercial grade, adjusting the

silica to the desired percentage by the addition of silica sand, after allowing for the silica present as impurity in the lime and fluorspar. Magnesia present as a normal impurity in a good grade of lime is not objectionable. Alumina present as a small amount of impurity is also not objectionable. Indeed, the addition of approximately 5% of alumina seems to be advantageous as it reduces somewhat the melting point of the desulphurizing slag. The above slag flows freely at 1200° C. and this property is very desirable for efficient desulphurization.

Molten pig iron high in sulphur (0.25%) has been subjected to the action of the lime-fluorspar-silica slag above referred to, at 1400° C. for one hour at atmospheric pressure in a refractory container composed of carbon in the form of graphite. The slag and molten pig iron were under strong reducing conditions and the desulphurizing vessel was arranged so as to prevent direct contact with the atmosphere or with combustion gases high in oxygen, carbon dioxide or water vapor. Under these conditions the slag picked up as much as 10.79% sulphur, and the pig iron had its sulphur content reduced to 0.03% sulphur, so that there was more than one hundred times as high a percentage of sulphur in the slag as in the pig iron.

In other cases in which the pig iron initially contained only about 0.03% sulphur, the sulphur content of the pig iron was reduced to 0.002% and the slag picked up 0.11% sulphur.

These good desulphurizing results can be still further improved if the pressure on the slag is reduced, for example to 380 millimeters of mercury, or below, and an agitating non-oxidizing gas is passed through the bath. The sulphur content of the iron may be reduced to less than one-half, or less than one-quarter, or even less than one-tenth of that in the iron before treatment according to the invention.

A study has been made of the use of sodium oxide, Na<sub>2</sub>O, in the form of slags containing this oxide or its compounds as a substitute for lime in desulphurizing slags. The desulphurizing action of these compounds of sodium oxide, for example sodium carbonate, on pig iron is well known and this alternative can be used. It is found, however, that Na<sub>2</sub>O is readily attacked by carbon and silicon in the pig iron at temperatures of 1450° C. or below. The reaction produces carbon monoxide, silica and sodium vapor. The latter is very effective in converting FeS into Na<sub>2</sub>S and thus desulphurizing the pig iron. The sodium vapor causes difficulty in the handling of soda slags, and the reaction must be managed in such a way as to limit the formation of volatile soda derivatives in order to avoid excessive loss as fume. It is possible to use slags containing Na<sub>2</sub>O combined with SiO<sub>2</sub> and/or Al<sub>2</sub>O<sub>3</sub> and other oxides to overcome volatilization loss incident to sodium carbonate. The revivification of soda slags to remove sulphur and permit reuse presents special difficulties not present in the case of lime slags.

Detailed reference to the steps necessary when soda slags are used is, therefore, omitted, and the discussion is generally confined to slags containing alkaline earth oxides as the preponderant active constituents. However, the use of slags containing Na<sub>2</sub>O or other alkali metal oxides as active desulphurizing ingredients, when used as substitutes for alkaline earth oxides such as lime as active ingredients, is included herein. In some cases desulphurizing slags may be used which employ lime or other alkaline earth oxides and

also soda or other alkali metal oxides in combination.

The quantity of oxides of the type  $R_xO$  in the initial slag should exceed 30% for best results.

Due to the cheapness and freedom from volatilization, it is preferable to use a lime slag, although such preference is subject to change under varying economic and metallurgical conditions.

In choosing the slag, it is desirable to have one which will be of low viscosity and workable at temperatures of 1400° C., and for this purpose, the slag should preferably be freely fluid at as low as 1200° C. or in some cases at 1300° C.

It is very advantageous to use a slag which shows a high ratio of sulphur concentration in the slag, after use, to sulphur concentration in the desulphurized or partially desulphurized pig iron.

Much latitude is offered in the choice of slag composition. In general the slag composition and pressure should be chosen so that a ratio of sulphur in the slag to sulphur in the iron should exceed 100:1 and preferably exceed 200:1.

As explained in detail below, it is often advantageous to employ a desulphurizing slag which can be revivified or treated to remove its sulphur so that it can be used over and over again. The lime slags referred to fulfill this requirement.

The desulphurizing slag, after it has picked up, for example, 12% sulphur, is revivified by removing sulphur from the slag until, for example, less than 1% sulphur remains. This revivified slag is then used repeatedly to desulphurize further quantities of molten pig iron.

#### Desulphurizing apparatus

In order to obtain the best desulphurizing action with many slags I have found that it is necessary to keep the temperature of the pig iron as high as possible. For example, laboratory experiments with a slag comprising 80 parts blast furnace slag, 10 parts lime, 10 parts fluorspar, treating a pig iron initially containing 0.16% sulphur at 1475° C. produced a slag containing 2.98% sulphur and pig iron containing 0.0095% sulphur with a ratio of the percentage of sulphur in slag to the percentage of sulphur in metal of 314:1. Using the same slag and pig iron at lower temperature, for example 1300° C., the resultant slag contained only 1.75% sulphur, the resultant pig iron contained 0.022% sulphur, and the ratio of the percentage of sulphur in slag to the percentage of sulphur in metal had fallen to 70:1.

To take advantage of this accentuated desulphurizing action at higher temperature, I place the desulphurizing vessel in a position adjoining the blast furnace. In this manner I avoid any temperature loss such as would occur if the molten iron from the blast furnace is first placed in a transfer ladle and then transported to a desulphurizing vessel located, for example, at the mixer in the steel making plant.

I have also found that the desulphurizing power of slags comprising large amounts of blast furnace slag is very sensitive to the ratio of lime to silica present in the slag. At equilibrium the desulphurizing power of these slags as measured by the ratio of sulphur in the slag to sulphur in the iron varies not as the ratio of lime to silica in the slag, but approximately as the logarithm to the base ten of the lime-silica ratio. In desulphurizing iron after its removal from the blast furnace, it is very important that the iron, as

it is transferred from furnace to desulphurizing vessel, be not contaminated by admixture of impurities containing silica. Many natural sources of contaminating silica are present at the blast furnace, such as the fireclay used in closing the blast furnace tap-hole, loam used in fettling the iron runners, and coke breeze used for covering the exposed surface of the molten iron in runners, etc. For best results these contaminations can be avoided by causing the molten iron to pass through a small tea-pot ladle or similar device just before it enters the desulphurizing vessel. In this way the siliceous impurities are separated and the desulphurizing slag is kept uniform with as high a ratio of lime to silica as intended.

Agitation of the desulphurizing slag and molten pig iron is necessary in order to cause the desulphurizing reaction to proceed with convenient speed. The present inventor has performed experiments without agitating the molten slag and molten pig iron. Figure 20 shows the rate of sulphur removal under certain fixed conditions, using a slag consisting of 40% blast furnace slag, 30% fluorspar and 30% burnt lime, without agitation.

In this figure the molten pig iron contained 0.07% sulphur at the beginning of the experiment. This iron was treated with desulphurizing slag of the composition just noted under deoxidizing conditions and freedom from air contamination, and samples of iron were withdrawn for chemical analysis at specified times. In Figure 20 the experimental data has been plotted in a curve showing, as the ordinate, the percentage of sulphur present in the iron, and, as the abscissa, the elapsed time for the reaction expressed in minutes per inch of depth of the metal bath.

The rate of sulphur removal is proportional to the depth of molten metal. From the curve it will be seen that, in order to lower the sulphur content from 0.07% to 0.005%, approximately 12 minutes are required for each one inch of depth of metal bath. In a customary pig iron ladle a depth of metal of 60 inches or more is to be expected. Thus for a depth of 60 inches, an elapsed time of 720 minutes or 12 hours would be required to desulphurize to the above extent. This time is too long for most operating conditions.

The rate of reaction can be speeded up appreciably by agitating the molten metal and/or the slag in order to produce relative motion between the slag and the metal at their point of contact, the so-called slag-metal interface. It is believed that the slow speed of desulphurization which is obtained in a quiet bath is due to the resistance which the sulphur encounters in the regions closely adjoining the slag-metal interface whilst passing from the metal to the slag. When contact is first established between the pig iron and the slag, the slag rapidly absorbs sulphur but the reaction soon slows down because, without agitation, the system approaches equilibrium only in the limited region which is not too far removed from the slag-metal interface. By providing a relative motion between the mass of the slag and the iron, thereby bringing fresh slag and iron into the zone adjacent to the slag-metal interface, it is possible to speed the removal of the sulphur. By continuing this process of relative motion the difficulties of slow speed operation as described above in quiet baths can be overcome. The present invention is concerned with agitation to produce relative motion between the slag and the metal in order to speed up the reaction and obtain a higher content of sulphur in the

slag and/or a lower content of sulphur in the iron than would otherwise be obtained.

Figure 1 illustrates a desulphurizing vessel 20 equipped with a mechanical agitating device for obtaining increased relative motion between the molten pig iron and the supernatant slag. Such a vessel might contain from 40 to 200 tons or more of molten pig iron. The slag layer might approximate 1% to 10% or more of the depth of the molten iron. The shape of the vessel is approximately circular or oval in cross section and the axis of symmetry, that is, the axis running perpendicular to the plane of circular or oval cross section, is vertical.

The axis of symmetry as referred to herein will be what is commonly called the major axis in the ordinary case. Where the ladle cross section is circular, it will be the axis of generation of the ladle.

The vessel is provided with a suitable steel shell 21 substantially gas tight and capable of protecting the contents from access of the atmosphere or other oxidizing gases. The refractory lining 22 consists preferably of carbon or magnesite bricks which have suitable resistance to the corrosive action of the ladle contents. In order to conserve heat, these refractory bricks may be backed up with refractories 23 having lower thermal conductivity, as for example fireclay brick having an appreciably larger percent of pore space than normal for such products. In some cases fireclay brick may also be used in direct contact with the contents of the ladle, as for example in the lower part where the slag does not come into contact with the fireclay refractories for long periods of time.

A roof or cover 24 is provided for the ladle. Fireclay or other suitable refractories 25 such as carbon or magnesite can be used in lining this roof. For best results a flat roof should be used and in such construction the refractory brick are best held in position by suspending them by hangers or other suitable means (not shown) from the external steel shell 26.

An opening 27 is provided for charging the molten iron and slag. Usually the slag will be charged before the molten iron although this is not always critical. The iron will be tapped from the blast furnace or other source of supply through a runner 28. In order to prevent silica and other undesirable impurities from entering the desulphurizing ladle, a skimming ladle 29 is provided. The iron leaves the runner 28 and enters the open top of the skimming ladle at 30. This ladle is provided with a dam or skimmer 31. The molten iron passes beneath this skimmer and the floating impurities are held back at 32. The exit end of the skimming ladle is provided with a cover 33 which keeps the atmosphere from the interior of the treatment ladle. After the desulphurizing ladle is properly filled, the source of molten iron is cut off at the runner. The iron still remaining in the skimming ladle is poured into the desulphurizing ladle by tilting the skimmer about the trunnion 34. Thereupon the skimming ladle and cover are removed and a suitable permanent cover 35 is placed on the ladle to cover the opening 27 as shown in Figure 1a.

An opening 36 is provided in the cover 24 of the ladle for an impeller 37. This impeller is preferably a self-contained unit having an electric motor 38 and speed reducer 39. The motor will preferably be of variable speed direct current motor producing an impeller speed of 50 to 200 revolutions per minute or more. The speed chosen

may vary with different installations. The impeller and its operating mechanism make a gas-tight seal with the cover 24 and may be removed as a unit from the desulphurizing vessel and a cover 40 substituted as shown in Figure 1a.

There are several advantages in employing a ladle whose axis of symmetry is vertical for desulphurizing pig iron. This makes it possible to locate the desulphurizing slag at the level of maximum ladle cross section with utilization of full ladle capacity. Thus the slag-metal interface is of maximum area for a convenient refractory structure. Refractory repairs and replacements are much easier in a ladle whose axis of symmetry is vertical than in one whose axis of symmetry is horizontal. In a normal ladle whose axis of symmetry is vertical, a larger proportion of the pig iron will be at relatively great depth in the ladle than in a ladle whose axis of symmetry is horizontal. Therefore in a ladle whose axis of symmetry is vertical, there is greater importance in securing efficient stirring and stirring which is effective from the standpoint of desulphurization.

Different types of impellers may be used to impart stirring primarily in a horizontal plane, but with an upward stirring component. Figure 2 shows a pumping type of impeller of circular cross section made suitably of carbon refractories. The body of the impeller 41 has pumping passages 42 extending diagonally upward and outward as shown. The number of pumping passages 42 is not critical. The effect of the pumping impeller is to lift molten metal from the bath into contact with the desulphurizing slag. The inlet 43 of the pumping impeller will preferably be located below the slag-metal interface 44 and the outlet 45 above the slag-metal interface, as shown, to cause distribution of molten metal directly into the slag. The level of the impeller 41 is made adjustable as required, by using any one of several different lengths of extensions 46. Extension 46 may be also made of carbon refractory or may be made of so-called sillimanite refractory or other high aluminous material. Figure 2a shows a different length of extension 46'. The impeller assembly is carried on the rotating shaft 47 which may be made of suitable heat resistant metal with a hollow interior 48 into which cooling air or other fluid is blown by a suitable pipe 49. The impeller, extension and shaft are desirably threaded to one another at 50 and 51.

Another form of impeller capable of lifting pig iron is shown in Figure 3. In this case the impeller head 41' is desirably made of carbon refractory. It is attached to the rotating mechanism by means of a sillimanite, cyanite or other extension 46''. The carbon refractory is machined to provide a spiral fluting 52. The impeller is mounted so that the spiral fluting preferably extends into the pig iron and below the slag-metal interface 44. The rotation of the stirrer produces a corresponding rotary movement in the slag and metal with which it is in contact. By virtue of the fluting, a vertical motion is also produced which preferably lifts the iron and the slag above the level which it would normally take if the fluting were absent. The effect of the pumping impeller is to lift the molten metal from the bath and bring it into better contact with the desulphurizing slag thereby exposing fresh slag-metal interfaces to speed up the sulphur removal.

An alternative apparatus for producing the required agitation is shown in Figures 4 and 5.

This consists of a rotating stirrer of carbon or other suitable refractory which is supported by a sillimanite extension 46 as shown in Figures 2 and 3. The stirrer 41<sup>2</sup> can be made from a round carbon electrode of suitable diameter, for example 10 inches to 15 inches or more if necessary. The round electrode can be machined to form a rectangular or other section 53 having one or more plane surface 54. For example, a rectangle 5 inches wide and 10 inches to 15 inches or more in length might be used. The stirrer is immersed in the slag and metal. By its rotation a corresponding rotary motion of the contents of the ladle is produced.

For better results two or more stirrers 41<sup>3</sup> and 41<sup>4</sup> may be used as shown in Figures 6 and 7. If two stirrers are used, they should be spaced so that the clearance between the rotating carbons should not be too great, as for example, a clearance of approximately 6 inches to 18 inches. These stirrers may rotate in the same direction or in opposite directions. If they are rotated in the same direction, the entire mass of liquid contents of the ladle will be given a corresponding rotating motion as shown by the arrows in Figure 7.

Where a plurality of stirrers are to be used as in Figures 6 and 7, improved results are obtained by having the stirrers effective at different levels in the bath. Thus in Figure 6 the stirrer 41<sup>3</sup> extends deeper into the bath than the stirrer 41<sup>4</sup>, the latter stirrer operating chiefly in the slag and not extending any great depth below the slag-metal interface. These two stirrers produce a relative movement between the slag and the metal, and also between respective portions of the metal.

In order to speed up the rate of reaction it is desirable to have a relative movement between the slag layer and the metal. The natural tendency would be for the slag layer and the metal layer to rotate together and the relative motion between the two would not be as great as desirable. Increased relative motion can be obtained by using the apparatus shown in Figures 8 and 9. A dam 55 is immersed in the slag layer and if desired, below the slag-metal interface 44. Any desired number of dams may be used. The effect of the dam is to impede the rotation of the slag whilst permitting a relatively unhampered rotation of the pig iron, thereby causing relative motion between the pig iron and the slag. The dam may if desired occupy the opening 27 when metal is not being charged, with suitable packings to exclude air.

Where there is considerable variation in the level of the pig iron, it is desirable to make the height of the dam adjustable so that the dam will always extend down to the slag-metal interface and also preferably slightly below the interface as shown. In Figures 10 and 11 I show a refractory dam 55' suitably of carbon refractory supported on a bracket 56 and adjustable as to height by an adjusting screw 57 threaded through the bracket and making thrust bearing connection with the dam 55'. To prevent the dam from rotating, a guide 58 extends from the dam through an opening in the bracket 56.

In some instances it is preferable to use a floating dam 55<sup>2</sup> as shown in Figure 12. This dam, preferably of carbon refractory, automatically adjusts itself with respect to the level of the slag-metal interface and its volume-weight may be adjusted by adding weights 59 to make it float with any desired degree of submergence. While the dam 55<sup>2</sup> may float freely, it is preferable to

flexibly restrain it, as by a refractory chain 60 anchored to the vessel 20 at 61. The structures of Figures 10 to 12 will be provided with a suitable gas-tight cover as shown in Figure 1.

- 5 To further promote better transfer of the impurities from the molten iron to the slag, the apparatus shown in Figures 13 and 14 can be applied either alone or in conjunction with the dam 55 and/or the two stirrers 41<sup>3</sup> and 41<sup>4</sup> as shown. 10 In this type of apparatus the refractory lining is constructed to form an inclined vane 62 extending around the ladle circumference from point 63 near the bottom to point 64 near the top and providing a vane shelf 65 which is a maximum at 63 15 and a minimum at 64. The vane 62 is capable of converting some of the rotary motion of the liquid iron in the ladle into vertical motion, thereby bringing the metal from the bottom of the ladle upward to establish contact with the supernatant slag. The rotatory action of the metal may be imparted by the stirrers 41<sup>3</sup> and 41<sup>4</sup> or in other suitable ways.

Instead of using the mechanical agitators for producing a rotary motion in the molten pig iron in the ladle, it is also possible to produce a rotary motion by means of electromagnetic action. By using polyphase alternating current to produce rotating magnetic fields in an iron core suitably placed around the periphery of the ladle, preferably at or below the slag-metal interface, the current induced by the alternating electromagnetic field in the molten metal contained in the ladle causes a rotary motion of the metal in the way that rotary motion is produced in a polyphase induction motor.

30 Figures 15 and 16 show such a polyphase stirring ladle having a winding 66 intended for three-phase alternating current, with phase field coils 67, 68 and 69 connected to a source at 70, 71 and 72 and connected together at 73 (Figure 15). Star connection is shown, but it will be evident that any suitable system of connections may be used. The winding is surrounded by an annular magnetic core 74 suitably slotted to receive the 35 winding as at 75 and desirably laminated. Low frequency alternating current at, for example, 25 to 100 cycles will preferably be used.

The device of Figures 15 and 16 will cause 40 simultaneous rotation of both the slag and the metal. To secure differential movement between the slag and the metal, a slag dam 55 of any desired type will desirably be used as shown in Figure 16; or an inclined vane 62 as also shown in this figure; or mechanical stirrers will be employed as shown at 41<sup>3</sup> and 41<sup>4</sup> in Figure 16, preferably causing the slag to rotate oppositely from the metal.

45 Figures 17 and 18 illustrate a variant electromagnetic stirring device. The desulphurizing vessel 20 is surrounded by a polyphase winding 76 of Gramme ring type, wound on an annular magnetic core 77, suitably laminated, and provided with magnetic poles 78. In the specific construction, a three-phase winding consists of phase coils 79, 80, and 81 connected in delta formation to three-phase lines 82, 83, and 84 from an alternating current source at commercial frequency. The magnetic core 77 and the poles 78 will desirably be assembled from separate units, fastened 50 together in any suitable manner.

The winding 76 and core 77 are very desirably inclined or canted with respect to the horizontal as shown in Figure 18, so that in addition to a horizontal rotary or whirling motion in the iron,

there will be a helical upward stirring component due to the inclination of the winding and core.

There will preferably be one coil and one pole for each phase, and, of course, the number of phases in the polyphase system may be varied. In general, the smaller the number of poles, the faster the stirring, other conditions being unchanged. It is very desirable to have the structural arrangement of the poles such that the flux from pole to adjoining pole will pass through a substantial portion of the iron bath and not merely through the wall of the ladle. It is preferable, therefore, to use a small number of poles, for example from two to six poles.

The ladle of Figures 17 and 18 is desirably provided with a slag dam 55 and with impellers 41<sup>3</sup> and 41<sup>4</sup>. While the iron whirls in upward helical paths, the whirling of the slag is retarded by the dam 55. The impellers 41<sup>3</sup> and 41<sup>4</sup>, which operate in the slag, will desirably rotate the slag oppositely from the rotation of the iron. For example, if the iron rotates in the direction of the arrow 85, the slag will preferably be rotated by the impellers in the opposite direction.

It will, of course, be understood that in Figures 15 to 18 the ladles will be provided with air tight closures.

Instead of a moving wave form of electromagnetic stirrer as shown in Figures 15 to 18, a pool surrounding coreless induction form of any well known type may be used. In Figure 1 an inductor coil 66 surrounds the upper portion of the metal bath adjacent the slag-metal interface. The neighboring structural parts of the ladle will desirably be made of non-magnetic metals or alloys or non-metallic materials. A suitable alternating current of low frequency, for example 25 to 100 cycles, will be connected to the coil 66. The coil will desirably carry a high wattless current due to resonance obtained through suitably connected condensers as well known in the art. In some respects the inductor coil stirring is undesirable as it is accompanied by considerable heat obtained at relatively high cost.

The ladles for containing the molten metal and slag to be rotated as described above should have a vertical axis of symmetry about which the rotation takes place. For example, the interior could be shaped in the form of a cylinder or inverted truncated cone. The major axis of the cylinder or cone stands approximately vertical and rotation occurs about this axis. It is not necessary that the cross section of the ladle on a plane at right angle to this axis of symmetry be circular. Indeed, it may be advantageous to use some other shape as for example an elliptical or oval section, thereby facilitating the formation of new areas of slag-metal interface as the metal rotates about its natural axis. For example, the oval cross section shown in Figure 19 when rotated by any of the means described turns about an axis located at the point 86. An element 87 of slag-metal interface is rotated by this motion to the position 87<sup>1</sup>. By so doing the area of the interface is increased. Further rotation causes the element to move to 87<sup>2</sup> with attendant decrease in area of the slag-metal interface. At position 87<sup>3</sup> the area is again increased. Thus a repeated formation of new areas of interface occurs by rotating the slag and metal in an oval shaped vessel.

An illustrative cycle of operations with reference particularly to Figure 1 is as follows: The desulphurizing ladle is charged through the opening 27 with the required amount of desulphurizing

slag from the pot 88. This desulphurizing slag may, for example, comprise 70 per cent of molten blast furnace slag previously withdrawn from the blast furnace, 20 per cent of burned lime and 10 per cent fluorspar. The blast furnace is tapped and about 150 tons of iron is transferred into the ladle 29. As described above, all siliceous contaminations should be removed from the flowing stream of iron by dams or skimming devices. The desulphurizing ladle and its charge is then closed against free access of air or oxygen to the interior. Desulphurizing is continued using agitation until the proper sulphur content of the iron has been obtained. For best results vacuum may be applied to the ladle, as through a vacuum connection 89.

After the desulphurizing reaction is completed, the slag is removed by tilting the ladle 29 about the axis 90 and allowing the slag to run out the opening 91 (suitably closed against air contamination when not in use) into the slag pot 88. Thereupon the ladle is tilted in the reverse direction about the axis 92 and the iron is poured through the tea-pot spout 93 (suitably sealed when not in use) into the transfer ladles 94. A symmetrical axis is also provided at 92' for pouring the entire ladle content, slag and iron, in emergency. Two or more transfer ladles 94 may be used if necessary and the stream of metal from the desulphurizing ladle can be interrupted by tilting the ladle 29 whilst a new transfer ladle is brought into position. It is important that any desulphurizing slag remaining in the desulphurizing ladle be kept from entering the transfer ladles 94. The inclined tea-pot spout 93 is effective to prevent this. If further precautions are necessary the small tea-pot skimmer ladle 95 can be placed just ahead of the transfer ladles 94.

With good agitation and efficient slags, a pig iron containing 0.015% sulphur or 0.010% sulphur or less may be obtained from a blast furnace product containing initially as much as 0.10% to 0.30% sulphur or more. The sulphur content of the slags may rise to 5% or 10% sulphur or more and a ratio of sulphur in slag to sulphur in the iron of 500:1 or 1000:1 and even 5000:1 or more, all depending upon the chosen conditions.

Of course, the processes and apparatus described herein may be used for the removal of sulphur from molten pig iron supplied by furnaces other than a blast furnace, as for example a cupola. The use for such purposes is expressly included herein.

In view of the invention and disclosure variations and modifications to meet individual whim or particular need will doubtless become evident to others skilled in the art, to obtain all or part of the benefits of my invention without copying the structure shown, and I, therefore, claim all such in so far as they fall within the reasonable spirit and scope of my invention.

Having thus described my invention what I claim as new and desire to secure by Letters Patent is:

1. The process of desulphurizing molten pig iron, which comprises treating molten pig iron under deoxidizing conditions in a closed space with a basic desulphurizing slag floating on the pig iron and projecting streams of molten pig iron upwardly into the slag at the slag-pig iron interface.

2. The process of desulphurizing molten pig iron, which comprises treating molten pig iron under deoxidizing conditions with a basic desulphurizing slag in a closed space, maintaining sub-

atmospheric pressure in the space and projecting streams of molten pig iron upwardly into the slag at the slag-pig iron interface.

3. The process of desulphurizing pig iron, which comprises electromagnetically whirling the iron in a generally horizontal rotary direction and maintaining a substantial body of molten desulphurizing slag on the iron while rotating the slag in a direction opposite to the direction of rotation of the iron.

4. The process of desulphurizing molten pig iron, which comprises electromagnetically whirling

ing the iron in a generally horizontal rotating path, imparting an upward stirring component to the iron and maintaining a substantial body of molten desulphurizing slag on the iron.

5. The process of desulphurizing molten pig iron, which comprises electromagnetically stirring molten pig iron in a helical path, tending to bring submerged metal to the surface, and maintaining a substantial body of molten desulphurizing slag on the iron.

RUSSELL PEARCE HEUER.